

## [54] PHOTOCOCONDUCTIVE COMPOSITION AND ELECTROPHOTOGRAPHIC LIGHT-SENSITIVE MATERIAL USING SAID COMPOSITION

[75] Inventors: Syun-ichi Kondo; Kenji Sano; Hideo Sato, all of Saitama, Japan

[73] Assignee: Fuji Photo Film Co., Ltd., Kanagawa, Japan

[21] Appl. No.: 472,305

[22] Filed: Mar. 4, 1983

## [30] Foreign Application Priority Data

Mar. 4, 1982 [JP] Japan ..... 57-33082

[51] Int. Cl.<sup>3</sup> ..... G03G 5/05; G03G 5/09

[52] U.S. Cl. ..... 430/83; 430/81

[58] Field of Search ..... 430/83, 81; 252/501.1

## [56] References Cited

## U.S. PATENT DOCUMENTS

3,617,271 11/1971 Poot ..... 430/81

## FOREIGN PATENT DOCUMENTS

28455 7/1974 Japan ..... 430/81

## OTHER PUBLICATIONS

Hoegl, "On Photoelectric Effects in Polymers and their Sensitization by Dopants", The Journal of Physical Chemistry, vol. 69, No. 3, Mar. 1965, pp. 755-766.

Primary Examiner—Mary F. Downey

Attorney, Agent, or Firm—Sughrue, Mion, Zinn, Macpeak and Seas

[57]

## ABSTRACT

A photoconductive composition comprising an organic photoconductive substance and at least one compound represented by the general formula (I) or (II)



wherein X is an alkyl group, a substituted alkyl group, an aryl group, a substituted aryl group, an alkoxy group, a substituted alkoxy group, an aryloxy group, n and m are each an integer of 1 or 2, and l and k are each an integer of from 1 to 4, and, optionally, a sensitizing dye capable of increasing the sensitivity of the organic photoconductive substance, and an electrophotographic light-sensitive material comprising a support having an electrically conductive surface and a layer of the photoconductive composition layer on the support. This electrophotographic light-sensitive material has sensitivity and superior stability with time.

19 Claims, No Drawings

**PHOTOCONDUCTIVE COMPOSITION AND  
ELECTROPHOTOGRAPHIC LIGHT-SENSITIVE  
MATERIAL USING SAID COMPOSITION**

**FIELD OF THE INVENTION**

The present invention relates to photoconductive compositions composed mainly of organic photoconductive substances, and electrophotographic light-sensitive materials bearing an electrophotographic light-sensitive layer which is made up of the composition. More particularly, the present invention relates to high sensitivity photoconductive compositions composed mainly of organic photoconductive substances and compounds represented by the general formula (I) or (II) as described hereinafter, and high sensitivity electrophotographic light-sensitive materials carrying an electrophotographic light-sensitive layer which is made up of the composition.

**BACKGROUND OF THE INVENTION**

As is well known, photoconductive substances for electrophotographic light-sensitive compositions include many organic compounds. Some of these organic compounds have been confirmed to have considerably high sensitivity. In fact, however, only a very limited number of organic photoconductive substances have been used in the preparation of electrophotographic materials.

Organic photoconductive substances have many superior properties compared with inorganic photoconductive substances, and therefore, may find many uses in the field of electrophotography. For example, transparent electrophotographic light-sensitive films, flexible electrophotographic light-sensitive films, those electrophotographic light-sensitive films which are light and easy to handle, and so forth can be prepared very advantageously using organic photoconductive substances. In addition, organic photoconductive substances have characteristics which could not be expected from the characteristics inorganic photoconductive substances e.g., film-forming properties during the production of electrophotographic light-sensitive materials, surface smoothness, and choice of the desired charging polarity in electrophotographic processes.

These organic photoconductive substances, however, have not yet been widely used in the field of electrophotography mainly because of their low sensitivity and poor film strength, although they have many excellent characteristics as described above.

Initially, low molecular heterocyclic compounds, nitrogen-containing aromatic compounds, various polymer type aromatic compounds, etc. have been extensively investigated as organic photoconductive substances. However, the sensitivity of these compounds must be increased to much higher levels, because even those organic photoconductive substances which are known to have the highest sensitivity do not have sufficient sensitivity to be put into practical use as such without the application of a sensitization treatment. For this reason, various sensitization methods have been studied. In the practical use of organic photoconductive substances, therefore, it is essential to select and employ a sensitization method which is most effective for them. It may safely be said that the industrial value of organic photoconductive substances is determined by the sensitization technique to be employed, i.e., by the increased sensitivity of the ultimate electrophotographic light-

sensitive material which is achieved by application of the sensitization technique.

Addition of Lewis acids is such a sensitization method. In this method, sensitization is achieved by the appearance of a new spectral sensitivity resulting from the formation of a donor/acceptor complex between Lewis acids and organic photoconductive substances.

All the systems comprising organic photoconductive substances, sensitizing dyes, and heretofore known Lewis acids have poor stability with the lapse of time and are not suitable for practical use.

**SUMMARY OF THE INVENTION**

An object of the invention is to provide photoconductive compositions which are highly sensitized, and have excellent stability with the lapse of time.

Another object of the invention is to provide electrophotographic light-sensitive materials which have high sensitivity and have excellent stability with the lapse of time.

It has now been found that addition of compounds represented by the general formula (I) or (II) as described hereinafter increases the light sensitivity of organic photoconductive substances and provides excellent stability with the lapse of time. Therefore, the above-described objects are achieved by using the compounds represented by the general formula (I) or (II).

The present invention provides as embodiments:

(1) a electrophotoconductive composition containing an organic photoconductive substance or substances and at least one compound represented by the general formula (I) or (II):



wherein X is an alkyl group, a substituted alkyl group, an aryl group, a substituted aryl group, an alkoxy group, a substituted alkoxy group, an aryloxy group, or a substituted aryloxy group, n and m are each an integer of 1 or 2, and 1 and k are each an integer of from 1 to 4;

(2) a photoconductive composition containing an organic photoconductive substance or substances, at least one compound represented by the general formula (I) or (II) as described above, and a sensitizing dye or dyes capable of increasing the sensitivity of the organic photoconductive substance or substances;

(3) an electrophotographic light-sensitive material comprising a support having an electrically conductive surface, and a photoconductive composition layer on the support, the photoconductive composition containing an organic photoconductive substance or substances and at least one compound represented by the general formula (I) or (II) as described above; and

(4) an electrophotographic light-sensitive material comprising a support having an electrically conductive

surface, and a photoconductive composition layer on the support, the photoconductive composition containing an organic photoconductive substance or substances, at least one compound represented by the general formula (I) or (II) as described above, and a sensitizing dye or dyes capable of increasing the sensitivity of the organic photoconductive substance or substances.

#### DETAILED DESCRIPTION OF THE INVENTION

Various organic photoconductive substances can be used in the invention. Preferred are those substances which can be dye-sensitized. Typical photoconductive substances are given below:

- (i) Polymeric organic photoconductive substances resulting from the polymerization of polycyclic aromatic or heterocyclic aromatic vinyl compounds containing  $\pi$ -electrons.

Typical examples of  $\pi$ -electron-containing nuclei constituting polymeric organic photoconductive substances include polycyclic aromatic hydrocarbon nuclei, e.g., naphthalene, anthracene, pyrene, perillene, acenaphthylene, phenylanthracene, and diphenylanthracene; heterocyclic aromatic compound nuclei, e.g., carbazole, indole, acridine, 2-phenylindole, and N-phenylcarbazole; and their halogen or lower alkyl-substituted derivatives. In the invention, vinyl polymers containing the above-described nuclei can be used as photoconductive substances. These vinyl polymers include vinyl polymers, such as polyvinyl naphthalene, polyvinyl anthracene, polyvinyl pyrene, polyvinyl perillene, polyacenaphthylene, polystyryl anthracene, polyvinyl carbazole, polyvinyl indole, and polyvinyl acridine, and copolymers of the vinyl compounds constituting the above-described vinyl polymers; vinyl ether polymers, such as polyanthryl methylvinyl ether, polypyrenyl methylvinyl ether, polycarbazolyl ethylvinyl ether, and polyindolyl ethylvinyl ether, and copolymers of the vinyl ether compounds constituting the above-described vinyl ether polymers; epoxy resins, such as polyglycidyl carbazole, polyglycidyl indole, and poly-p-glycidyl anthrylbenzene; homo- and copolymers of acrylic acid esters and methacrylic acid esters, for example, containing the above-described  $\pi$ -electron-containing nuclei as a substituent; and condensates of the above-described  $\pi$ -electron-containing compounds and formaldehyde.

Suitable polyvinyl carbazoles include poly-N-vinyl carbazole, poly-N-vinyl carbazole derivatives containing a substituent or substituents, e.g., an aryl group, an alkylaryl group, an amino group, an alkylamino group, a dialkylamino group, an arylamino group, a diarylamino group, a N-alkyl-N-arylarnino group, a nitro group, and a halogen atom, on the carbazole ring (these compounds are hereinafter referred to as "poly-N-vinyl carbazole substituted derivatives"), and N-vinyl carbazole or substituted N-vinyl carbazole copolymers.

Exemplary N-vinyl carbazole copolymers which can be used are those copolymers containing at least 50 mol% of the N-ethylene carbazole constitutional repeating unit having the formula (III):



wherein Q is the same substituent as defined for the above-described poly-N-vinyl carbazole substituted derivatives. Preferred examples of other repeating units constituting N-vinyl carbazole copolymers are 1-phenylethylene, 1-cyanoethylene, 1-cyano-1-methylethylene, 1-chloroethylene, 1-(alkoxycarbonyl)ethylene, and 1-alkoxycarbonyl-1-methylethylene, the repeating units being derived from styrene, acrylonitrile, methacrylonitrile, vinyl chloride alkyl acrylate, and alkyl methacrylate, respectively. The alkyl group of the alkoxy carbonyl group can be an alkyl group containing from 1 to 18 carbon atoms, including a methyl group, an ethyl group, a hexyl group, a dodecyl group, an octadecyl group, and a 4-methylcyclohexyl group. The terms "constitutional repeating unit" as used herein is the same as defined in *Kobunshi (Polymer Journal)*, vol. 27, pp. 345-359 (1978) (Japanese version of *Pure and Applied Chemistry*, vol. 48, pp. 375-385 (1976)).

Of these polymeric organic photoconductive substances, poly-N-vinyl carbazole, poly-N-vinyl carbazole substituted derivatives containing the above-described substituents, and N-vinyl carbazole or substituted N-vinyl carbazole copolymers are most preferred.

#### (ii) Aromatic tertiary amino compounds

35 Triphenylamine, N,N-dibenzylaniline, diphenylbenzylamine, N,N-di(p-chlorobenzyl)aniline, di( $\beta$ -naphthyl)benzylamine, tri(p-tolyl)amine, and diphenylcyclohexylamine

#### (iii) Aromatic tertiary diamino compounds

40 N,N,N',N'-Tetrabenzyl-p-phenylenediamine, N,N,N',N'-tetra(p-chlorobenzyl)-p-phenylenediamine, N,N,N',N'-tetramethyl-p-phenylenediamine, N,N,N',N'-tetrabenzyl-m-phenylenediamine, 45 N,N,N',N'-tetramethylbenzidine, N,N,N',N'-tetrabenzylbenzidine, N,N,N',N'-tetraphenyl-p-phenylenediamine, N,N,N',N'-tetraphenyl-m-phenylenediamine, 1,1-bis[4-(dibenzylamino)phenyl]ethane, 1,1-bis[4-(dibenzylamino)phenyl]propane, 1,1-bis[4-(dibenzylamino)-phenyl]butane, 1,1-bis[4-(dibenzylamino)phenyl]2-methylpropane, 2,2-bis[4-(dibenzylamino)phenyl]propane, 2,2-bis[4-(dibenzylamino)phenyl]butane, 1,1-bis 50 4-[di(m-methylbenzylamino)phenyl]propane, bis[p-(dimethylamino)phenyl]phenylmethane, bis[p-(dimethylamino)phenyl]phenylmethane, bis[4-(dibenzylamino)phenyl]methane, bis[4-[di(p-chlorobenzyl)amino]phenyl]methane, 1,1-bis[p-(dimethylamino)-phenyl]-1-phenylethane, 4,4'-benzylidenebis(N,N-dimethyl-m-toluidine), 4',4"-bis(diethylamino)-2,6-dichloro-2',2"-dimethyltriphenylmethane, bis[4-(diethylamino)-2-methylphenyl]- $\alpha$ -naphthylmethane, 4',4"-bis(dimethylamino)-2-chloro-2',2"-dimethyltriphenylmethane, 1,1-bis[p-(diethylamino)phenyl]-1-phenylethane, 1,1-diphenyl-5,5-bis[4-(diethylamino)-2-methylphenyl]-1,3-pentadiene, 1,1-diphenyl-3,3-bis[4-(diethylamino)-2-methylphenyl]-propane, bis[4-(dibenzylamino)phenyl]ether, bis[4-(diethylamino)-phenyl]ether, bis[4-(dibenzylamino)phenyl]sulfide, 2,2-

60 65

bis[4-(di-p-tolylamino)phenyl]propane, 1,1-bis[4-(di-p-tolylamino)phenyl]-1-phenylethane, and bis[4-dibenzylamino]phenyl]diphenylmethane

(iv) Aromatic tertiary triamino compounds

Tris[4-(diethylamino)phenyl]methane, and 1,1-bis[4-(diethylamino)-2-methylphenyl]-1-[4-(dimethylamino)-phenyl]methane

(v) Condensates

Condensates of aldehydes and aromatic amines, such as a condensate of acetaldehyde and  $\alpha$ -naphthylamine, a condensate of formaldehyde and N-ethylaniline, condensates of tertiary aromatic amines, such as triphenylamine, and aromatic halides, and condensates of poly-p-phenylene-1,3,4-oxadiazole, formaldehyde, and condensed polycyclic aromatic compounds, such as 3,6-dimethyl carbazole.

(vi) Metal-containing compounds

2-Mercaptobenzothiazole lead salt, 2-mercaptobenzothiazole zinc salt, 2-mercaptobenzothiazole copper salt, 2-mercaptobenzoxazole lead salt, 2-mercaptop-5-phenylbenzoxazole lead salt, 2-mercaptop-6-methoxybenzimidazole lead salt, 8-hydroxyquinoline magnesium salt, 8-hydroxyquinoline aluminum salt, 8-hydroxyquinoline lead salt, 7-benzyl-8-hydroxyquinoline copper salt, and 2-hydroxy-4-methylazobenzene copper salt,

(vii) Heterocyclic compounds

(a) Pyrazoline derivatives

1,3,5-Triphenylpyrazoline, 1-phenyl-3-[p-(dimethylstyryl)-5-[p-(dimethylamino)phenyl]pyrazoline, 1,5-diphenyl-3-styrylpyrazoline, 1,3-diphenyl-5-styrylpyrazoline, 1,3-diphenyl-5-[p-(dimethylamino)phenyl]pyrazoline, and 1,3-diphenyl-5-(2-furyl)pyrazoline

(b) 1,2,4-Triazine derivatives

3-[p-(dimethylamino)phenyl]-5,6-bis(p-dimethoxyphenyl)-1,2,4-triazine, 3-[p-(dimethylamino)phenyl]-5,6-di(2-pyridyl)-1,2,4-triazine, 3-[p-(dimethylamino)phenyl]-5,6-di(p-ethoxyphenyl)-1,2,4-triazine, 3-[p-(diethylamino)phenyl]-5,6-bis(p-methoxyphenyl)-1,2,4-triazine, and 3-[p-(diethylamino)phenyl]-5,6-bis(p-ethoxyphenyl)-1,2,4-triazine

(c) Quinazoline derivatives

2,4-Diphenylquinazoline, 2-phenyl-4-p-tolylquinazoline, 2 phenyl-4-[4-(dimethylamino)phenyl]quinazoline, 2-phenyl-4-styrylquinazoline, and 2,4-diphenylbenzo[h]quinazoline

(d) Benzofuran derivatives

6-Hydroxy-2-phenyl-3-[4-(dimethylamino)phenyl]benzofuran, 6-hydroxy-2,3-di(4-methoxyphenyl)benzofuran, and 2,3,5,6-tetra(4-methoxyphenyl)benzo[1,2-b:5,4-b]difuran

(e) Oxadiazole derivatives

2,5-Bis[4-(dimethylamino)phenyl]-1,3,4-oxadiazole, 2,5-bis[4-(diethylamino)phenyl]-1,3,4-oxadiazole, and 2,5-bis[4-(isoamylamino)phenyl]-1,3,4-oxadiazole

All the compounds represented by the general formula (I) or (II) can be synthesized by the method described in *Beilsteins Handbuch der Organischen Chemie*, vol. 10, page 149.

The alkyl or alkoxy group indicated by X in the general formulae (I) and (II) can be a straight or branched alkyl or alkoxy group containing from 1 to 22 carbon atoms.

Substituents for substituted alkyl and alkoxy groups indicated by X in the general formulae (I) and (II) include a halogen atom, e.g., a chlorine atom, a bromine atom, and a fluorine atom, a cyano group, a nitro group, a phenyl group, and a tolyl group. Thus, the substituted alkyl or alkoxy group, can be a straight or branched alkyl or alkoxy group containing from 1 to 22 carbon atoms and with from 1 to 3 substituents as described above bound thereto.

10 The aryl or aryloxy group represented by X may be monocyclic or bicyclic (of the two-ring condensed type). Typical examples include a phenyl group, a naphthyl group, a phenoxy group, and a naphthoxy group.

15 Substituents for the substituted aryl and aryloxy groups include a halogen atom, e.g., a chlorine atom, a bromine atom, and a fluorine atom, a cyano group, a nitro group, a straight or branched alkyl group containing from 1 to 5 carbon atoms, a straight or branched alkoxy group containing from 1 to 5 carbon atoms, an

20 alkoxy carbonyl group containing a straight or branched alkyl group having from 1 to 5 carbon atoms, and a phenyl or naphthyl group containing from 1 to 3 acyl groups, with the acyl group containing a straight or branched alkyl group having from 1 to 5 carbon atoms.

25 The compounds of the general formula (I) or (II) as used herein have great advantages in that they increase the light sensitivities of organic photoconductive substances, they have good compatibility with organic photoconductive substances, particularly poly-N-vinyl carbazole, poly-N-vinyl carbazole substituted derivatives, and copolymers of N-vinyl carbazole or substituted N-vinyl carbazoles, and they produce electrophotographic light-sensitive layers (photoconductive composition layers) of electrophotographic light-sensitive

30 materials, having good film properties (e.g., films are uniform, tough, and flexible, and have a great adhesivity to supports).

Typical examples of the compounds represented by the general formula (I) include ethyl p-hydroxybenzoate, ethyl m-hydroxybenzoate, ethyl o-hydroxybenzoate, methyl p-hydroxybenzoate, butyl p-hydroxybenzoate, propyl p-hydroxybenzoate, phenyl p-hydroxybenzoate, naphthyl p-hydroxybenzoate, chloroethyl p-hydroxybenzoate, p-tolyl p-hydroxybenzoate, p-ethylphenyl p-hydroxybenzoate, diethyl 2-hydroxyterephthalate, diethyl 2-hydroxyisophthalate, ethyl 2,4-dihydroxybenzoate, 4-acetylphenol, p-hydroxybenzophenone, and p-hydroxyphenyl ethyl ketone.

Typical examples of the compounds represented by the general formula (II) include 5-ethoxycarbonyl-1-naphthol, 3-ethoxycarbonyl-1-naphthol, 5-methoxycarbonyl-1-naphthol, 5-butoxycarbonyl-1-naphthol, 5-propoxycarbonyl-1-naphthol, 5-phenoxy carbonyl-1-naphthol, 4-ethoxycarbonyl-2-naphthol, 6-ethoxycarbonyl-2-naphthol, 5-acetyl-1-naphthol, 5-propionyl-1-naphthol, 5-benzoyl-1-naphthol, 4-acetyl-2-naphthol, and 4-benzoyl-2-naphthol.

In the invention, the sensitivity of photoconductive compositions comprising organic photoconductive substances and compounds of the general formula (I) or (II) can be further increased by adding thereto sensitizing dyes capable of increasing the sensitivity of the organic photoconductive substances.

For this purpose, known sensitizing dyes which are used in the dye-sensitization of organic photoconductive substances can be used. Typical examples of such sensitizing dyes are described in *Society of Photographic Scientists and Engineers*, 19, 60-64 (1975), *Applied Optics*,

Suppl., 3, 50 (1969), U.S. Pat. Nos. 3,037,861, 3,250,615, 3,712,811, British Pat. No. 1,353,264, *Research Disclosure*, #10938 (109, May 1973, page 62), U.S. Pat. Nos. 3,141,700, 3,938,994, Japanese Patent Application (OPI) Nos. 14560/81, 14561/81, 29586/81, 29587/81, 65885/81 (the term "OPI" is used herein to mean a "published unexamined Japanese Patent Application"), Japanese Patent Application No. 114259/80, and Japanese Patent Application (OPI) No. 35141/81.

From these known sensitizing dyes and other dyes capable of increasing the sensitivity of polymeric organic photoconductive substances, any suitable dye can be selected and used.

Suitable examples of the above-described sensitizing dyes are given below:

Triphenylmethane Dyes, such as Brilliant Green, Victoria Blue B, Methyl Violet, Crystal Violet, and Acid violet 6B; Rhodamines, such as Rhodamine B, Rhodamine 6G, Rhodamine G Extra, Sulfo Rhodamine B, and Fast Acid Eosine G; xanthene dyes, such as Eosine S, Eosine A, Erythrosine, Phloxine, Rose Bengal, and Fluorescein; thiazine dyes, such as Methylene Blue; acridine dyes, such as Acridine Yellow, Acridine Orange, and Trypaflavin; quinoline dyes, such as pinacyanol, and cryptocyanine; quinone and ketone dyes, such as Alizarine, Alizarine Red S, and quinizarin; cyanine dyes; chlorophyll; arylmethane dyes, such as Violet Fuchsine, Erythrosine 2Na, Rhodamine B 500, Fanal Pink B, Rhodamine 6 GDN, and Auramine; polymethylene dyes, such as 3,3-diethylthiacyanine iodide; 30 azo dyes such as Eriochrome Blue-Black R; azomethine dyes, such as bis(p-dimethylaminobenzal)azine; carbonyl dyes, such as Solway Ultra Blue B, and Alizarine Cyanin Green GWA; heterocyclic compounds, such as N,N-pentamethylenebis(benzthiazole) perchlorate; phthalocyanine dyes, such as Segnale, Light, Turquoise NB; and pyrylium dyes, such as 2,6-di-tert-butyl-4-(2,6-di-tert-butyl-4H-thiopyran-4-indenemethyl)-thiapyrylium salt, 2,6-di-tert-butyl-4-[(2,6-di-tert-butyl-4H-thiopyran-4-indene)propen-1-yl]thiapyrylium salt, 40 2,6-diphenyl-4-(4-diethylaminophenyl)thiapyrylium salt, and 2,6-di-tert-butyl-4-(4-diethylaminostyryl)-thiapyrylium salt.

These sensitizing dyes are added in amounts sufficient to sensitize organic photoconductive substances, and therefore, the amount of sensitizing dye added varies with the types of organic photoconductive substance and sensitizing dye. In general, sensitizing dyes can be added in an amount ranging between about 0.01 and 100 parts by weight, preferably between about 0.1 and 30 parts by weight, per 100 parts by weight of organic photoconductive substance.

The photoconductive composition of the invention may contain, if necessary, known structure agents, improving film strength plasticizers, dyes, pigments, etc., within the ranges not deteriorating the composition characteristics.

Structure agents which can be used include cyanoethyl cellulose, nitrile rubber, polycarbonate of bisphenol A, linear polyesters, styrene-butadiene copolymers, and vinylidene-acrylonitrile copolymers. Plasticizers which can be used include chlorinated biphenyls, epoxy resins, triphenylmethane compounds, cumarone resins, and low molecular weight xylene resins.

In preparing the photoconductive composition of the invention, the above-described two or more components, and ingredients which are to be added, if present, are dispersed or dissolved in a desired ratio to prepare a

dispersion or uniform solution, the dispersion or uniform solution is coated on a suitable support, and the common solvent is removed, for example, by vaporization. Depending on the purpose for which the photoconductive composition is used, the dispersion or uniform solution may be used as such without completely removing the solvent. The thus-prepared photoconductive composition solution is coated on a suitable support having an electrically conductive surface and dried to form a photoconductive layer. Depending on the use, an adhesive layer and so forth may be employed.

Suitable solvents or dispersants which can be used in the preparation of coating solutions include benzene, toluene, xylene, chlorobenzene, dichlorobenzene, dichloroethane, trichloroethane, cyclohexanone, tetrahydrofuran, dioxane, etc., and mixtures thereof, those solvents capable of dissolving or dispersing therein polymeric organic photoconductive substances, sensitizing dyes, compound represented by the general formula (I) or (II), and additives to be added, if present, can be used.

The proportion of the compound represented by the general formula (I) or (II) in the photoconductive composition is determined in relation to the amount of the organic photoconductive substance contributing to photoconductive insensitivity. The amount of the compound represented by the general formula (I) or (II) used is from about 0.1 to 100 parts by weight, and preferably from 0.5 to 30 parts by weight, per 100 parts by weight of the organic photoconductive substance. Addition of the compound of the general formula (I) or (II) above or below the above-specified limits results in a reduction in sensitivity of the resulting photoconductive composition and an increase in residual potential.

For supports with an electrically conductive surface, it is sufficient that at least the surface is electrically conductive. In more detail, drums and sheets made of metals, such as aluminum, copper, iron, and zinc, and paper, plastics, glass, etc., whose surface has been rendered electrically conductive by, for example, vacuum-depositing metals, such as aluminum, copper, zinc, and indium, vacuum-depositing electrically conductive metallic compounds, such as  $In_2O_3$  and  $SnO_2$ , laminating a metallic foil, and dispersing carbon black, an electrically conductive metallic compound (e.g.,  $In_2O_3$  and  $SnO_2$ ) powder, metallic powder, or the like in binder polymers and coating the resulting dispersions, can be used.

Addition of the compounds represented by the general formula (I) or (II) to organic photoconductive substances permits production of electrophotographic light-sensitive films which are highly sensitized and are stable with time.

It is also possible for the photoconductive composition of the invention to be ground to fine particles, dispersed in insulating solvents, and processed by an electrophoresis image-forming photographic process described in, for example, U.S. Pat. Nos. 3,384,565 (corresponding to Japanese Patent Publication No. 21781/68), 3,384,488 (corresponding to Japanese Patent Publication No. 37125/72), and 3,510,419 (corresponding to Japanese Patent Publication No. 36079/71), to form images.

The following examples are given to illustrate the invention in greater detail. Unless otherwise indicated herein all parts, percents, ratios and the like are by weight.

## EXAMPLE 1

One gram of poly-N-vinyl carbazole (PVCz) was dissolved in 20 ml of 1,2-dichlorethane, and 25 mg of 2,6-di-tert-butyl-4-[4-(N-methyl-N-2-cyanoethylamino)styryl]thiapyrylium tetrafluoroborate was added to the resulting solution.

The thus-prepared solution was coated on a 100  $\mu\text{m}$  thick polyethylene terephthalate (PET) film having a 60 nm thick  $\text{In}_2\text{O}_3$  vacuum-deposited layer thereon (i.e., 10 was used.

15 were prepared (examples of this invention). The sensitivity of the photoconductive layer was measured for the thus-prepared Electrophotographic Films Nos. 1 to 15 i.e., the exposure amount ( $E_{50}$ ) at which the initial potential (500 V) was reduced to one-half ( $\frac{1}{2}$ ) by attenuation, and the exposure amount ( $E_{90}$ ) at which the initial potential (500 V) was reduced to one-tenth (1/10) were measured. The results are shown in Table 1 below. As a light source, a 630 nm monochromatic light

TABLE 1

| Electrophotographic Film No. | Compound Represented by General Formula (I) or (II) | Amount (parts by weight) | $E_{50}$ (erg/cm <sup>2</sup> ) | $E_{90}$ (erg/cm <sup>2</sup> ) |
|------------------------------|-----------------------------------------------------|--------------------------|---------------------------------|---------------------------------|
| 1 (comparative example)      | —                                                   | —                        | 65                              | 430                             |
| 2                            |                                                     | 1                        | 48                              | 311                             |
| 3                            |                                                     | 5                        | 36                              | 218                             |
| 4                            |                                                     | 1                        | 50                              | 310                             |
| 5                            |                                                     | 5                        | 35                              | 214                             |
| 6                            |                                                     | 1                        | 47                              | 298                             |
| 7                            |                                                     | 5                        | 35                              | 210                             |
| 8                            |                                                     | 1                        | 55                              | 340                             |
| 9                            |                                                     | 5                        | 40                              | 230                             |
| 10                           |                                                     | 1                        | 50                              | 310                             |
| 11                           |                                                     | 5                        | 38                              | 226                             |
| 12                           |                                                     | 1                        | 47                              | 300                             |
| 13                           |                                                     | 5                        | 35                              | 210                             |
| 14                           |                                                     | 1                        | 52                              | 320                             |
| 15                           |                                                     | 5                        | 37                              | 220                             |

PET film made electrically conductive with  $\text{In}_2\text{O}_3$ ), and 55 then, dried to remove the solvent, forming a 5  $\mu\text{m}$  thick photoconductive layer (an electrophotographic light-sensitive layer). In this way, Electrophotographic Film No. 1 (comparative example) was prepared.

To a portion of the above-prepared solution were 60 added the compounds represented by the general formula (I) or (II) as shown in Table 1 below in the amount also shown in Table 1 (per 100 parts by weight of PVCz) to prepare a series of solutions. Each solution was coated on the same PET film made electrically 65 conductive with  $\text{In}_2\text{O}_3$  as above and dried to remove the solvent, forming a 5  $\mu\text{m}$  thick photoconductive layer. In this way, Electrophotographic Films Nos. 2 to

## EXAMPLE 2

Electrophotographic Films Nos. 16 (comparative example), 17 and 18 (examples of this invention), 19 (comparative example), and 20 and 21 (examples of this invention) were prepared in the same manner as in the preparation of the Electrophotographic Films Nos. 1 and 2 in Example 1 except that 25 mg of 2,6-di-tert-butyl-4-[4-(N,N-dichloroethylamino)styryl]-thiapyrylium tetrafluoroborate and 25 mg of Rhodamine B (C.I. #45170) were used in place of 25 mg of 2,6-di-tert-butyl-4-[4-(N-methyl-N-2-cyano-

thylaminostyryl]thiapyrylium tetrafluoroborate. The sensitivity of these electrophotographic films was measured using the same method as in Example 1. The results are shown in Table 2 below.

## EXAMPLE 3

Electrophotographic Films Nos. 22 (comparative example), and 23 and 24 (examples of this invention) were prepared in the same manner as in the preparation of the Electrophotographic Films Nos. 1 and 2 in Example 1 except that a PET film having a  $\text{SnO}_2$  fine powder/gelatin layer, prepared by the method described in Examples 1 and 2 of Japanese Patent Application No. 47665/80, was used in place of the PET film rendered electrically conductive with  $\text{In}_2\text{O}_3$ . The sensitivity of these electrophotographic films was measured using the same method as in Example 1. The results are shown in Table 2 below.

TABLE 2

| Electrophotographic Film No. | Sensitizing Dye                                                                      | Compound Represented by General Formula (I) or (II)                                 | Amount (parts by weight) | $E_{50}$ (erg/cm <sup>2</sup> ) | $E_{90}$ (erg/cm <sup>2</sup> ) |
|------------------------------|--------------------------------------------------------------------------------------|-------------------------------------------------------------------------------------|--------------------------|---------------------------------|---------------------------------|
| 16 (comparative example)     | 2,6-di-tert-butyl-4-[4-N,N-dichloroethyl-amino]styryl]thiapyrylium tetrafluoroborate |                                                                                     | —                        | 60                              | 412                             |
| 17                           | "                                                                                    |   | 1                        | 47                              | 308                             |
| 18                           | "                                                                                    |    | 5                        | 34                              | 200                             |
| 19 (comparative example)     | Rhodamine B                                                                          |                                                                                     | —                        | 140                             | 1020                            |
| 20                           | "                                                                                    |   | 1                        | 84                              | 680                             |
| 21                           | "                                                                                    |  | 5                        | 70                              | 520                             |
| 22 (comparative example)     | Same as in No. 1                                                                     |                                                                                     | —                        | 66                              | 441                             |
| 23                           | "                                                                                    |  | 1                        | 48                              | 310                             |
| 24                           | "                                                                                    |  | 5                        | 36                              | 212                             |



15 wherein X is an alkyl group, a substituted alkyl group, an aryl group, a substituted aryl group, an alkoxyl group, a substituted alkoxyl group, an aryloxyl group, or a substituted aryloxyl group, n and m each represent

15

10

10

15

15

20

20

25

25

30

30

35

35

40

40

45

45

50

50

55

55

60

60

65

65

70

70

75

75

80

80

85

85

90

90

95

95

100

100

105

105

110

110

115

115

120

120

125

125

130

130

135

135

140

140

145

145

150

150

155

155

160

160

165

165

170

170

175

175

180

180

185

185

190

190

195

195

200

200

205

205

210

210

215

215

220

220

225

225

230

230

235

235

240

240

245

245

250

250

255

255

260

260

265

265

270

270

275

275

280

280

285

285

290

290

295

295

300

300

305

305

310

310

315

315

320

320

325

325

330

330

335

335

340

340

345

345

350

350

355

355

360

360

365

365

370

370

375

375

380

380

385

385

390

390

395

395

400

400

405

405

410

410

415

415

420

420

425

425

430

430

435

435

440

440

445

445

450

450

455

455

460

460

465

465

470

470

475

475

480

480

485

485

490

490

495

495

500

500

505

505

510

510

515

515

520

520

525

525

530

530

535

535

540

540

545

545

550

550

555

555

560

560

565

565

570

570

575

575

580

580

585

585

590

590

595

595

600

600

605

605

610

610

615

615

620

620

625

625

630

630

635

635

640

640

645

645

650

650

655

655

660

660

665

665

670

670

675

675

680

680

685

685

690

690

695

695

700

700

705

705

tertiary aromatic amine and an aromatic halide, a condensate of poly-p-phenylene-1,3,4-oxadiazole formaldehyde and, a condensed polycyclic aromatic compound, a metal-containing compound, or a heterocyclic compound.

6. The electrophotoconductive composition as claimed in claim 1, wherein the substituents for the substituted alkyl and alkoxy group represented by X in the general formula (I) and (II) are a halogen atom, a cyano group, a nitro group, a phenyl group, or a tolyl group and wherein the substituted alkyl or alkoxy group comprises a straight or branched chain alkyl or alkoxy group containing from 1 to 22 carbon atoms and with from 1 to 3 substituents as set forth above bound thereto; said aryl or aryloxy group represented by X in the general formula (I) and (II) is a monocyclic or bicyclic aryl or aryloxy group; said substituents for the substituted aryl or aryloxy group are a halogen atom, a cyano group, a nitro group, a straight or branched chain alkyl group containing from 1 to 5 carbon atoms, a straight or branched chain alkoxy group containing from 1 to 5 carbon atoms, an alkoxy carbonyl group containing a straight or branched chain alkyl group having from 1 to 5 carbon atoms, or a phenyl or naphthyl group containing from 1 to 3 acyl groups, each acyl group containing a straight or branched chain alkyl moiety having from 1 to 5 carbon atoms therein.

7. The electrophotoconductive composition as claimed in claim 1, wherein said compound of the general formula (I) is ethyl p-hydroxybenzoate, ethyl m-hydroxybenzoate, ethyl o-hydroxybenzoate, methyl p-hydroxybenzoate, butyl p-hydroxybenzoate, propyl p-hydroxybenzoate, phenyl p-hydroxybenzoate, naphthyl p-hydroxybenzoate, chloroethyl p-hydroxybenzoate, p-tolyl p-hydroxybenzoate, p-ethylphenyl p-hydroxybenzoate, diethyl 2-hydroxyterephthalate, ethyl 2,4-dihydroxybenzoate, 4-acetylphenol, p-hydrobenzophenone or p-hydroxyphenyl ethyl ketone and said compound of the general formula (II) is 5-ethoxycarbonyl-1-naphthol, 3-ethoxycarbonyl-1-naphthol, 5-methoxycarbonyl-1-naphthol, 5-butoxycarbonyl-1-naphthol, 5-propoxycarbonyl-1-naphthol, 5-phenoxy carbonyl-1-naphthol, 4-ethoxycarbonyl-2-naphthol, 6-ethoxycarbonyl-2-naphthol, 5-acetyl-1-naphthol, 5-propionyl-1-naphthol, 5-benzoyl-1-naphthol, 4-acetyl-2-naphthol or 4-benzoyl-2-naphthol.

8. The electrophotoconductive composition as claimed in claim 2, wherein said organic photoconductive substance is a polymeric organic photoconductive substance comprising the polymerization product of polycyclic aromatic or heterocyclic vinyl compounds containing  $\pi$ -electrons, an aromatic tertiary amino compound, an aromatic tertiary diamino compound, an aromatic tertiary triamino compound, a condensate of an aldehyde and an aromatic amine, a condensate of a tertiary aromatic amine and an aromatic halide, a condensate of poly-p-phenylene-1,3,4-oxadiazole and formaldehyde, a condensed polycyclic aromatic compound, a metal-containing compound, or a heterocyclic compound.

9. The electrophotoconductive composition as claimed in claim 2, wherein the substituents for the substituted alkyl and alkoxy group represented by X in the general formula (I) and (II) are a halogen atom, a cyano group, a nitro group, a phenyl group, or a tolyl group and wherein the substituted alkyl or alkoxy group comprises a straight or branched chain alkyl or

alkoxy group containing from 1 to 22 carbon atoms and with from 1 to 3 substituents as set forth above bound thereto; said aryl or aryloxy group represented by X in the general formula (I) and (II) is a monocyclic or bicyclic aryl or aryloxy group; and substituents for the substituted aryl or aryloxy group are a halogen atom, a cyano group, a nitro group, a straight or branched chain alkyl group containing from 1 to 5 carbon atoms, a straight or branched chain alkoxy group containing from 1 to 5 carbon atoms, an alkoxy carbonyl group containing a straight or branched chain alkyl group having from 1 to 5 carbon atoms, or a phenyl or naphthyl group containing from 1 to 3 acyl groups, each acyl group containing a straight or branched chain alkyl moiety having from 1 to 5 carbon atoms therein.

10. The electrophotoconductive composition as claimed in claim 2, wherein said compound of the general formula (I) is ethyl p-hydroxybenzoate, ethyl m-hydroxybenzoate ethyl o-hydroxybenzoate, methyl p-hydroxybenzoate, butyl p-hydroxybenzoate, propyl p-hydroxybenzoate, phenyl p-hydroxybenzoate, naphthyl p-hydroxybenzoate, chloroethyl p-hydroxybenzoate, p-tolyl p-hydroxybenzoate, p-ethylphenyl p-hydroxybenzoate, diethyl 2-hydroxyterephthalate, diethyl 2-hydroxyisophthalate, ethyl 2,4-dihydroxybenzoate, 4-acetylphenol, p-hydrobenzophenone or p-hydroxyphenyl ethyl ketone and said compound represented by the general formula (II) is 5-ethoxycarbonyl-1-naphthol, 3-ethoxycarbonyl-1-naphthol, 5-methoxycarbonyl-1-naphthol, 5-butoxycarbonyl-1-naphthol, 5-propoxycarbonyl-1-naphthol, 5-phenoxy carbonyl-1-naphthol, 4-ethoxycarbonyl-2-naphthol, 6-ethoxycarbonyl-2-naphthol, 5-acetyl-1-naphthol, 5-propionyl-1-naphthol, 5-benzoyl-1-naphthol, 4-acetyl-2-naphthol or 4-benzoyl-2-naphthol.

11. The electrophotoconductive composition as claimed in claim 2, wherein said sensitizing dye is a triphenylmethane dye, a rhodamine dye, a xanthene dye, a thiazine dye, an acridine dye, a quinoline dye, a quinone and keone dye, a cyanine dye, chlorophyll, an arylmethane dye, a polymethine dye, an azo dye, an azomethine dye, a carbonyl dye, a heterocyclic compound dye, a phthalocyanine dye, or a pyriliump dye.

12. The electrophotographic light-sensitive material as claimed in claim 3, wherein said organic photoconductive substance is a polymeric organic photoconductive substance comprising the polymerization product of polycyclic aromatic or heterocyclic vinyl compounds containing  $\pi$ -electrons, an aromatic tertiary amino compound, an aromatic tertiary diamino compound, an aromatic tertiary triamino compound, a condensate of an aldehyde and an aromatic amine, a condensate of a tertiary aromatic amine and an aromatic halide, a condensate of poly-p-phenylene-1,3,4-oxadiazole formaldehyde, and a condensed polycyclic aromatic compound, a metal-containing compound, or a heterocyclic compound.

13. The electrophotographic light-sensitive material as claimed in claim 3, wherein the substituents for the substituted alkyl and alkoxy group represented by X in the general formula (I) and (II) are a halogen atom, a cyano group, a nitro group, a phenyl group, or a tolyl group and wherein the substituted alkyl or alkoxy group comprises a straight or branched chain alkyl or alkoxy group containing from 1 to 22 carbon atoms and with from 1 to 3 substituents as set forth above bound thereto; said aryl or aryloxy group represented by X in the general formula (I) and (II) is a monocyclic or bicyclic

clic aryl or aryloxy group; said substituents for the substituted aryl or aryloxy group are a halogen atom, a cyano group, a nitro group, a straight or branched chain alkyl group containing from 1 to 5 carbon atoms, a straight or branched chain alkoxy group containing from 1 to 5 carbon atoms, an alkoxy carbonyl group containing a straight or branched chain alkyl group having from 1 to 5 carbon atoms, or a phenyl or naphthyl group containing from 1 to 3 acyl groups, each acyl group containing a straight or branched chain alkyl moiety having from 1 to 5 carbon atoms therein.

14. The electrophotographic light-sensitive material as claimed in claim 3, wherein said compound of the general formula (I) is ethyl p-hydroxybenzoate, ethyl m-hydroxybenzoate, ethyl o-hydroxybenzoate, methyl p-hydroxybenzoate, butyl p-hydroxybenzoate, propyl p-hydroxybenzoate, phenyl p-hydroxybenzoate, naphthyl p-hydroxybenzoate, chloroethyl p-hydroxybenzoate, p-tolyl p-hydroxybenzoate, p-ethylphenyl p-hydroxybenzoate, diethyl 2-hydroxyterephthalate, diethyl 2-hydroxyisophthalate, ethyl 2,4-dihydroxybenzoate, 4-acetylphenol, p-hydrobenzophenone or p-hydroxyphenyl ethyl ketone and said compound of the general formula (II) is 5-ethoxycarbonyl-1-naphthol, 3-ethoxycarbonyl-1-naphthol, 5-methoxycarbonyl-1-naphthol, 5-butoxycarbonyl-1-naphthol, 5-propoxycarbonyl-1-naphthol, 5-phenoxy carbonyl-1-naphthol, 4-ethoxycarbonyl-2-naphthol, 6-ethoxycarbonyl-2-naphthol, 5-acetyl-1-naphthol, 5-propionyl-1-naphthol, 5-benzoyl-1-naphthol, 4-acetyl-2-naphthol or 4-benzoyl-2-naphthol.

15. The electrophotographic light-sensitive material as claimed in claim 4, wherein said organic photoconductive substance is a polymeric organic photoconductive substance comprising the polymerization product of polycyclic aromatic or heterocyclic vinyl compounds containing  $\pi$ -electrons, an aromatic tertiary amino compound, an aromatic tertiary diamino compound, an aromatic tertiary triamino compound, a condensate of an aldehyde and an aromatic amine, a condensate of a tertiary aromatic amine and an aromatic halide, a condensate of poly-p-phenylene-1,3,4-oxidiazole formaldehyde and, a condensed polycyclic aromatic compound, a metal-containing compound, or a heterocyclic compound.

16. The electrophotographic light-sensitive material as claimed in claim 4, wherein the substituents for the substituted alkyl and alkoxy group represented by X in the general formula (I) and (II) are a halogen atom, a cyano group, a nitro group, a phenyl group, or a tolyl

5 10

group and wherein the substituted alkyl or alkoxy group comprises a straight or branched chain alkyl or alkoxy group containing from 1 to 22 carbon atoms and with from 1 to 3 substituents as set forth above bound thereto; said aryl or aryloxy group represented X in the general formula (I) and (II) is a monocyclic or bicyclic aryl or aryloxy group; said substituents for the substituted aryl or aryloxy group are a halogen atom, a cyano group, a nitro group, a straight or branched chain and alkyl group containing from 1 to 5 carbon atoms, a straight or branched chain alkoxy group containing from 1 to 5 carbon atoms, an alkoxy carbonyl group containing a straight or branched chain alkyl group having from 1 to 5 carbon atoms, or a phenyl or naphthyl group containing from 1 to 3 acyl groups, each acyl group containing a straight or branched chain alkyl moiety having from 1 to 5 carbon atoms therein.

17. The electrophotographic light-sensitive material as claimed in claim 4, wherein said compound of the general formula (I) is ethyl p-hydroxybenzoate, ethyl m-hydroxybenzoate, ethyl o-hydroxybenzoate, methyl p-hydroxybenzoate, butyl p-hydroxybenzoate, propyl p-hydroxybenzoate, phenyl p-hydroxybenzoate, naphthyl p-hydroxybenzoate, chloroethyl p-hydroxybenzoate, p-tolyl p-hydroxybenzoate, p-ethylphenyl p-hydroxybenzoate, diethyl 2-hydroxyterephthalate, diethyl 2-hydroxyisophthalate, ethyl 2,4-dihydroxybenzoate, 4-acetylphenol, p-hydrobenzophenone or p-hydroxyphenyl ethyl ketone and said compound of the general formula (II) is 5-ethoxycarbonyl-1-naphthol, 3-ethoxycarbonyl-1-naphthol, 5-methoxycarbonyl-1-naphthol, 5-butoxycarbonyl-1-naphthol, 5-propoxycarbonyl-1-naphthol, 5-phenoxy carbonyl-1-naphthol, 4-ethoxycarbonyl-2-naphthol, 6-ethoxycarbonyl-2-naphthol, 5-acetyl-1-naphthol, 5-propionyl-1-naphthol, 5-benzoyl-1-naphthol, 4-acetyl-2-naphthol or 4-benzoyl-2-naphthol.

18. The electrophotographic light-sensitive material as claimed in claim 4, wherein said sensitizing dye is a triphenylmethane dye, a rhodamine dye, a xanthene dye, a thiazine dye, an acridine dye, a quinoline dye, a quinone and ketone dye, a cyanine dye, chlorophyll, an arylmethane dye, a polymethine dye, an azo dye, an azomethine dye, a carbonyl dye, a heterocyclic compound dye, a phthalocyanine dye, or a pyriidium dye.

19. The electrophotographic light-sensitive material as claimed in claim 3, wherein said support is or has a surface of a metal or a paper, plastic or glass whose surface has been rendered electrically conductive.

\* \* \* \* \*